

Aug. 25, 1925.

1,551,495

E. LIONNE

FLEXIBLE MATERIAL HAVING TEMPORARY PROTECTING MEANS FOR ITS SURFACE

Filed May 24, 1920

Cellulose film.



Fig. 1.



Fig. 2.



Fig. 3.



Fig. 4.



Fig. 5.

Inventor.  
Ernest Lionne

Ernest Lionne  
Attest

## UNITED STATES PATENT OFFICE.

ERNEST LIONNE, OF NEEDHAM HEIGHTS, MASSACHUSETTS.

## FLEXIBLE MATERIAL HAVING TEMPORARY PROTECTING MEANS FOR ITS SURFACE.

Application filed May 24, 1920. Serial No. 383,674.

*To all whom it may concern:*

Be it known that I, ERNEST LIONNE, a citizen of the Republic of France, residing at Needham Heights, in the county of Norfolk and State of Massachusetts, have invented an Improvement in a Flexible Material Having Temporary Protecting Means for Its Surface, of which the following is a specification.

10 This invention relates to a novel fabric or similar flexible material which is adapted to enter into the composition of a manufactured product as a shoe.

In the manufacture of such a product as 15 a shoe many manufacturing operations are performed and the shoe undergoes much handling before it is finally finished and in condition to be sold.

The outer surfaces of the shoe by reason 20 of the various manufacturing operations and the handling, become soiled and must be cleaned before the shoe is salable. Attempts have been made to protect the surface of the shoe during the manufacturing 25 process as by stitching a paper or the like covering to the edges of the pieces as the vamp, uppers, etc., entering into the shoe or applying other temporary protective coverings adapted to receive the soil and at 30 the proper time removing the protective covering with the soil thereon thereby to expose the protected surface in its original state of cleanliness.

Such temporary protective coverings have 35 been applied to the individual pieces entering into the manufacture of the finished product or to the surface of the product at an intermediate stage of manufacture.

The object of this invention is to provide 40 a novel fabric or the like in large sheets or in the web having a protective covering for that surface adapted subsequently to be exposed in the finished product in which pieces of the novel fabric are incorporated.

45 The protective covering of the novel fabric is adapted to adhere to the smaller pieces cut therefrom during the manufacture of the article and receive the soil resulting from the manufacturing operations. At the 50 proper time the protective covering is adapted to be removed or stripped from the body of the fabric in the manufactured product thereby to expose the protected surface in its original state of cleanliness.

55 The novel fabric, as canvas in the web

with the protective covering thereon, or leather in whole skins or sides with the protective covering thereon, is adapted to be sold to shoe and other manufacturers who will cut from the web or sheets the 60 smaller pieces or shapes to be incorporated in the shoe or other product. At the end of the manufacturing operation the protective cover will be removed and thrown away.

The protective covering may comprise 65 any one of a number of materials or substances which will present a relatively smooth outer face, so that it will not become easily abraded, will be flexible and pliable to bend with the body of the fabric 70 without becoming broken or becoming detached from the surface, will be tough to resist unintentional tearing, extensible when such characteristic is desirable, and will be 75 cheap.

While I may employ, for the temporary protective covering, any of a number of previously prepared sheets having suitable characteristics, I prefer to employ a protective covering formed as a film by coating over the surface to be protected with a film producing solution such as pyroxyline solution and subsequently remove the solvent from the coating to form the sheet or film. The film may be deposited thereon to 85 any suitable thickness best adapted to the requirements of the particular article or product made from the novel material.

One of the characteristics of my invention is that the protective coating or film shall 90 be relatively non-adherent to the surface covered by it in order that it may be readily removed. The pyroxyline film formed by the evaporation of the solvent from the solution will be by itself very adherent to the 95 fabric surface and will cling thereto so strongly that it can not be removed with facility. I, therefore, initially apply to the surface of the fabric of the material to be protected an initial coating adapted to receive the film producing solution and to which the film will adhere to a greater or less degree. The initial coating is in itself substantially non-adherent to the surface of the fabric. At least it will be substantially 100 non-adherent as compared with the adhesiveness of the film itself to the fabric.

I prefer to employ, among a number of compositions well adapted to form the non-adherent coating, a composition formed of 110

5 a pigment in a finely divided state, as kaolin, china clay, aluminum oxide or hydrate and the like; a binder which may be a gum as gum tragacanth, dextrine and the like; and a vehicle as water, benzol and the like.

The proportions of a composition well adapted for my purpose may comprise

|          | Parts. |
|----------|--------|
| 10 Water | 100    |
| Gum      | 2      |
| Pigment  | 40     |

15 or in such other suitable proportions as to provide proper, and relatively small, adhesency of the desired pulverulent coating formed thereby to the specific material to which protection is given.

20 The composition is applied uniformly on the surface of the material by suitable means as a coating knife and to the proper thickness. Preferably the coating is relatively thin so that the composition does little more than fill the interstices of the fabric 25 and does not extend above the surface of the material to any appreciable degree. The proportion of the composition and the ingredients of the composition will be so arranged that when the new fabric is finally 30 completed the outer coating or the film will have the proper degree of adhesency. I find in some instances that it may be advisable initially to wet the fabric and apply the non-adherent coating to the wetted fabric 35 whereby to assist in regulating the thickness of the coating.

After the non-adherent coating is applied it is dried and the fabric is in readiness 40 for further coating applications. The next layer, or the film producing solution from which the next layer is formed, may be applied directly on top of the non-adherent coating and in many instances this will be done. In some instances, however, I prefer 45 to apply to the surface of the dried non-adherent coating a solution containing gum and water which may be in the proportion of water 100 parts, gum 2 parts. This coating will be relatively thin and will serve to 50 condition the non-adherent coating to receive the film producing solution by filling or sealing over the pores in the non-adherent, pulverulent coating.

55 After the conditioning coating has been applied and dried the film producing solution is applied.

The film producing solution preferably 60 comprises a cellulosic solution, as a pyroxyline or other colloidal solution, but may comprise any solution adapted to form a film which will be relatively tough and tenacious, tear and wear-resisting, flexible and pliable to bend with the body-portion of the fabric or other material to which it is applied, and 65 present a relatively smooth outer surface

adapted to receive the soil of the manufacturing operations. As contrasted with the non-adherent, pulverulent coating, which is adapted to have but slight tenacity or ability to resist rupture and is relatively brittle, 70 and the particles composing it but weakly adherent to each other, the outer soil-receiving coating or film is adapted to be non-pulverulent, tough and tenacious and tear and wear-resisting, and extensible when 75 needed.

The solution adapted to form such a coating is applied over the conditioning coating by suitable means, as a coating knife, to form a film or coating of suitable thickness, 80 and the coating is dried by suitable means, as by drying rollers or by drying chambers. The novel material is now prepared and may be formed into a roll or otherwise arranged and is in condition to be cut up into 85 proper pieces and shapes which will be formed into some manufactured product.

It will be noted that the protective covering is formed in two distinctive layers each having different characteristics. The 90 initial coating is formed from a composition in which the main component, the pigment, is in suspension and the coating formed thereby is pulverulent. The substance forming the final coating is deposited from 95 a solution and the coating is tough and tenacious and presents a smooth surface.

The pieces cut from the coated fabric are adapted to be sewed to other pieces or otherwise formed into the finished product with 100 the coating thereon; and the coating receives the soil of the manufacturing operations. When the article is finished or when such a stage of manufacture has been 105 reached that it is desirable to remove the coating, the coating may be cut by a knife and an edge thereof raised, which edge is grasped and the outer film stripped from the surface in relatively large pieces. The film carries with it a considerable proportion of 110 the non-adherent pulverulent coating, which adheres thereto. The remainder of the pulverulent coating is in a more or less powdery form and is removed from the surface of the fabric by mechanical means as by a 115 revolving brush. The surface of the fabric is thereby exposed in its original state of cleanliness.

If the surface of the material to be protected is white then the pigment entering 120 into the composition of the non-adherent coating will be white also; and if the surface is of a different color then the pigment will be such as to match the color of the surface whereby the protective coating will 125 not in itself stain the surface of the material to be protected.

Fig. 1 is a perspective detail illustrating the various protective layers super-imposed 130 on the fabric.

Fig. 2 is a view similar to Fig. 1, with the conditioning layer absent.

Fig. 3 is a detail illustrating the protective covering partially stripped from the 5 fabric and showing the non-adherent coating clinging to the film and also to the fabric.

Fig. 4 is a detail illustrating the surface of the fabric in its cleaned state after the protective coating has been removed.

Fig. 5 is a detail illustrating the protective coating applied to a canvas material having a water proof backing strip permanently adherent thereto.

15 In the figures the fabric is represented by 10, the non-adherent coating by 50, the conditioning coating by 51 and the outermost coating or film by 52. For some purposes it may not be necessary to employ intermediate or conditioning coating and Fig. 2 illustrates a section of the new material in which the outer coating or film 52 is applied directly on top of the non-adherent coating 50.

25 Canvas entering into the manufacture of shoes usually is made partially water proof by cementing a backing strip to that face adapted to be innermost in the finished article with an adhesive rubber cement; and the 30 backing strip is adapted to be permanently united with the fabric by such cement.

My protective coating is well adapted to be applied to such material, and is illustrated in Fig. 5 in which the canvas 10 has 35 the layer of rubber cement 53 and the backing cloth 54 on one surface and the non-adherent coating 50 and the protecting film 52 on the other surface.

Fig. 3 illustrates a section of the protective coating partially removed from the body of the material and shows the manner in which the non-adherent coating is removed, part of the non-adherent coating clinging to the film covering and part clinging 45 to the surface of the fabric. After the outermost film with a large proportion of the non-adherent coating clinging thereto has been removed that portion of the non-adherent coating remaining on the surface 50 of the fabric is removed in powdery form by mechanical means as a revolving brush having relatively stiff bristles.

While I have illustrated my invention applied more specifically to canvas or similar 55 textile fabric yet it also will be applied to leather and other material in essentially the same manner, modified, however, to adapt the invention to the specific material employed.

60 I claim:

1. As a new product of manufacture a flexible material in large sheets or in the web having a temporary protective covering for a surface thereof comprising a sheet of material which is flexible to bend with the ma-

terial without rupture, and tough to resist unintentional tearing, and a pulverulent binder weakly uniting said protective covering to said material by which said protective covering is removably adherent to the 70 surface of the material, and adapted to adhere to small pieces cut from the large sheets and be subsequently removed from said pieces by mechanical means to expose the protected surface in its original state of 75 cleanliness.

2. As a new product of manufacture, a flexible material in large sheets or in the web, having a temporary protecting covering for a surface thereof comprising a tenacious and flexible sheet of material uniformly applied to the surface, and a pulverulent binder weakly uniting said protecting covering to said flexible material by which said protective covering is temporarily adherent to the surface and to the surface of small pieces cut from the large sheet, said pulverulent binder being sufficiently adherent to flex and bend with the material without being detached therefrom 90 and removable therefrom with said protective covering in pieces by mechanical means.

3. As a new product of manufacture a flexible material in the large sheets or in the web comprising a flexible body portion and temporary surface protecting means therefor comprising a flexible, colloidal sheet, and pulverulent means uniformly attaching it to the surface of the body portion admitting of its detachment therefrom in 100 pieces.

4. As a new product of manufacture a flexible material in large sheets or in the web comprising a body portion and temporary protective means for its surface 105 comprising a filler of pulverulent material uniformly applied over the surface to fill the interstices thereof characterized by the particles composing said filler weakly adhering to each other and to the surface of the body portion, a conditioning coating of a substance to fill the pores of said pulverulent filler applied uniformly over the surface of the pulverulent filler, and a flexible protective sheet uniformly applied over 110 the surface of the conditioning coating.

5. A flexible material having temporary protecting means for its surface comprising a surface covering of a pulverulent material characterized by the particles composing it having the color of the surface to be protected and relatively weakly adherent to each other and to the surface of the material, and a flexible protective coating superimposed upon and relatively strongly 120 adherent to the pulverulent surface covering, said temporary protective means characterized by a considerable portion of the pulverulent covering adhering to the flexible protective coating and removable with 125 130

- the pulverulent covering and the remainder of the pulverulent covering adhering to the surface of the material and removable therefrom by mechanical means.
- 5 6. A flexible textile material having temporary protecting means for its surface comprising an initial protective coating weakly adherent to the surface of the material and a final coating comprising a film of cellulosic material superimposed over the surface of the initial coating strongly adherent to said initial coating.
- 10 7. A flexible material having temporary protecting means for its surface comprising an initial protective pulverulent coating weakly adherent to the surface of the material, and a final coating superimposed on the surface of the initial coating comprising a film of cellulosic material strongly adherent to said initial coating.
- 15 8. The method of temporarily protecting the surface of a flexible material which consists in applying an intermediate weak and frangible coating to the surface, drying the coating, and applying an outer coating of a film-forming material to the dried intermediate coating, and drying said outer coating.
- 20 9. The method of temporarily protecting the surface of a flexible material in large sheets or in the web which consists in coating the surface of the material with a composition containing a liquid carrier and a pigment in suspension in the carrier, drying the coating to remove the carrier and leave a friable layer of pigment upon the surface, coating the dried friable layer with a film-producing solution, and drying the second coating to deposit a tenacious and adherent film on the dried first coating.
- 25 10. The method of temporarily protecting the surface of a flexible material in large sheets or in the web which consists in coating the surface of the material with a liquid composition containing a pigment in suspension, drying the coating to remove the carrier for the pigment, coating the surface of the dried coating with a conditioning solution containing a pore-closing substance for the pigment coating, drying the conditioning coating, coating the dried conditioning coating with a film producing solution, and drying the last-named coating to deposit a film superimposed over the previous coatings.
- 30 35 40 45 50 55
- In testimony whereof, I have signed my name to this specification.
- ERNEST LIONNE.